



US005110977A

**United States Patent** [19]

Wilson et al.

[11] **Patent Number:** 5,110,977[45] **Date of Patent:** May 5, 1992

[54] **ESTER-CONTAINING QUATERNARY AMMONIUM SALTS AS ADHESION IMPROVING TONER CHARGE AGENTS**

[75] Inventors: **John C. Wilson; Lawrence P. DeMejo**, both of Rochester; **Alexandra Bermel**, Spencerport, all of N.Y.

[73] Assignee: **Eastman Kodak Company**, Rochester, N.Y.

[21] Appl. No.: 479,774

[22] Filed: **Feb. 14, 1990**

[51] Int. Cl.<sup>5</sup> ..... C07C 69/75; C07C 69/76; G03G 9/06; G03G 9/08

[52] U.S. Cl. ..... 560/1; 560/110; 560/7; 560/61; 430/104; 430/105; 430/106; 430/107; 430/108; 430/109; 564/282; 564/283; 564/284; 554/91; 554/110; 554/103

[58] Field of Search ..... 430/110, 106, 107, 108; 564/282, 283, 284; 560/1, 110

[56]

**References Cited****U.S. PATENT DOCUMENTS**

|           |         |             |         |
|-----------|---------|-------------|---------|
| 3,873,583 | 3/1975  | Walz        | 260/404 |
| 4,190,717 | 2/1980  | Suzuki      | 526/62  |
| 4,299,898 | 11/1981 | Williams    | 430/106 |
| 4,323,634 | 4/1982  | Jadwin      | 430/110 |
| 4,587,269 | 5/1986  | Thomas, Jr. | 521/38  |
| 4,840,863 | 6/1989  | Otsu        | 430/110 |

**FOREIGN PATENT DOCUMENTS**

0321363 6/1989 European Pat. Off. .

*Primary Examiner*—Joseph L. Schofer

*Assistant Examiner*—Fred Zitomer

*Attorney, Agent, or Firm*—Dressler, Goldsmith, Shore, Sutker & Milnamow, Ltd.

[57]

**ABSTRACT**

Toner particles comprising a polyester binder and a charge control agent are provided wherein such agent is a quaternary ammonium salt having one or more ester-containing moieties. Such an ester-containing salt causes toner particles to display lower fusing temperature, improved paper adhesion indexes, and improved polyester binder compatibility compared to nonesterified salts.

1 Claim, No Drawings

ESTER-CONTAINING QUATERNARY  
AMMONIUM SALTS AS ADHESION IMPROVING  
TONER CHARGE AGENTS

FIELD OF THE INVENTION

This invention is in the field of ester containing quaternary ammonium salts having utility as charge control agents for toners that also serve as adhesion promoters between toner and receiver sheets and as toner fusing temperature reducers.

BACKGROUND OF THE INVENTION

In the art of making and using toner powders, charge control agents are commonly employed to adjust and regulate the triboelectric charging capacity and/or the electrical conductivity characteristics thereof. Many different charge control agents are known which have been incorporated into various binder polymers known for use in toner powders. However, the need for new and improved toner powders that will perform in new and improved copying equipment has resulted in continuing research and development efforts to discover new and improved charge control agents.

Of potential interest are substances which not only serve as toner powder charge control agents, but also function as agents that provide additional results or effects. Such multi-functionality not only offers the potential for achieving cost savings in the manufacture and use of toner powders but also offers the potential for achieving toner powders with performance capabilities not heretofore known.

Charge control agents that contain either incorporated ester groups or incorporated quaternary ammonium salt groups are known ("Research Disclosure No. 21030" Volume 250, October, 1981, published by Industrial Opportunities, Ltd., Homerville, Havant, Hampshire, P091EF, United Kingdom) but charge control agents that contain both ester groups and quaternary ammonium groups in the same molecule are unknown, so far as now known.

SUMMARY OF THE INVENTION

This invention is directed to toner powders comprising a polymeric matrix phase which has dispersed therein at least one quaternary ammonium salt having incorporated therein at least one ester containing moiety that is bonded through an alkylene linking group to a quaternary ammonium nitrogen atom.

When incorporated into toner powders, such quaternary ammonium salts not only function as charge control agents, but also as toner powder fusing temperature depressants and paper adhesion promoters. These salts are preferably dispersed in the polymeric binder matrix phase comprising the core or body portion of a toner particle. These salts appear to have greater compatibility with polyester resins than prior art charge control agents that contain only an ester group or a quaternary ammonium group.

Toner powders containing these salts incorporated into the polymeric binder thereof can be used for producing developed toned images on a latently imaged photoconductor element, for transfer of the toned image from the photoconductor element to a receiver sheet, and for heat fusion of the toned image on the receiver, while employing processes and processing

conditions heretofore generally known to the art of electrophotography.

Various other advantages, aims, features, purposes, embodiments and the like associated with the present invention will be apparent to those skilled in the art from the present specification taken with the accompanying claims.

DETAILED DESCRIPTION

(A) Definitions

The term "particle size" as used herein, or the term "size", or "sized" as employed herein in reference to the term "particles", means volume weighted diameter as measured by conventional diameter measuring devices, such as a Coulter Multisizer, sold by Coulter, Inc. Mean volume weighted diameter is the sum of the mass of each particle times the diameter of a spherical particle of equal mass and density, divided by total particle mass.

The term "glass transition temperature" or "T<sub>g</sub>" as used herein means the temperature at which a polymer changes from a glassy state to a rubbery state. This temperature (T<sub>g</sub>) can be measured by differential thermal analysis as disclosed in "Techniques and Methods of Polymer Evaluation", Vol. 1, Marcel Dekker, Inc., N.Y., 1966.

The term "melting temperature" or "T<sub>m</sub>" as used herein means the temperature at which a polymer changes from a crystalline state to an amorphous state. This temperature (T<sub>m</sub>) can be measured by differential thermal analysis as disclosed "Techniques and Methods of Polymer Evaluation".

The term "onset of fusing temperature" as used herein is relation to a toner powder means the lowest temperature at which a high density solid area patch developed with this toner exhibits good adhesion to paper as determined by the adhesion index and crack and rub tests. The crack and rub test involves fusing a toner patch onto paper, folding the patch and brushing the loose toner away, and evaluating the width of the crack. The adhesion index test involves adhering a metal block to a toner patch and measuring the energy required to cause interfacial failure between the toner layer and its contacting substrate by collision of a pendulum with the metal block. The term "ester compatibility" as used herein has reference to the capacity of a thermoplastic polymer, such as one usable in the manufacture of toner powders, to blend with an additive material which is an ester group containing quaternary ammonium salt compound.

(B) Quaternary Ammonium Salts

This invention is directed to quaternary ammonium salts of the formula:



wherein R<sub>1</sub> is alkyl, aryl, and



where

R<sub>5</sub> is arylene or alkylene;  
R<sub>2</sub> is alkyl, aryl or aralkyl or alkylene;  
R<sub>3</sub> is alkyl, aryl, aralkyl or



R<sub>4</sub> is alkyl, aryl or aralkyl;  
X is (CH<sub>2</sub>)<sub>n</sub> or arylene;  
Z<sup>⊖</sup> is an anion; and  
n is an integer from 2 to 6.

As used herein, the term "alkyl" includes straight and branched chain alkyl groups and cycloalkyl groups.

As used herein, the term anion refers to negative ions such as m-nitrobenzenesulfonate, tosylate, tetraphenylborate, dicyanamide, chloride, etc.

As used herein, the term aryl includes phenyl, naphthyl, anthryl and the like.

As used herein, the term arylene includes phenylene, naphthalene, and the like.

As used herein, the term aralkyl includes benzyl, naphthylmethyl and the like.

Alkyl and aryl groups can be unsubstituted or substituted with a variety of substituents such as alkoxy, halo or other groups.

Presently preferred quaternary ammonium salts are those of the formula



wherein

R<sub>1</sub> is cyclohexyl or phenyl;  
R<sub>2</sub> and R<sub>3</sub> are methyl;  
R<sub>4</sub> is benzyl;  
Z<sup>⊖</sup> is m-nitrobenzenesulfonate; and  
n is 2.

The quaternary ammonium salts of the present invention can also be pendant groups from polymeric backbones in which case R<sub>1</sub> has the formula:



wherein R<sub>6</sub> is hydrogen or alkyl and x is >1.

### (C) Synthesis

Compounds of Formula (1) can be prepared by any convenient route. One general route is to acylate a N,N-di(lower alkyl) amino lower alkanol with an acid chloride to produce the corresponding (N,N-di(lower alkyl)amino) alkyl esters which are subsequently quaternized with a reactive aliphatic or aromatic halide. The quaternary ammonium compound is converted to the desired anion by a metathesis or ion exchange reaction with a reactive alkali metal aryl sulfonate or other acid salt.

Preferably, the acid chloride is either benzoyl chloride or cyclohexanecarbonylchloride, while the hydroxylamine is either 2-(N,N-dimethyl)aminoethanol or

N-methyldiethanolamine. In place of the acid chloride, the corresponding carboxylic acid can be employed.

One convenient and presently preferred procedure for such an ester preparation is to prepare a basic aqueous solution of the tertiary amino alkanol. To this solution is slowly added a solution of the acid chloride in a water immiscible organic solvent, methylene chloride being presently preferred. The addition is preferably accompanied by rapid stirring. The mole ratio of amine to total added acid chloride is preferably about 1:1. The ensuing reaction is exothermic, and, after the reaction is complete, stirring is preferably continued for a time period, such as at least about 1/2 hour. The organic layer is then separated, washed with water and dried, preferably over MgSO<sub>4</sub> or the like, and concentrated. The product is typically an oil which can be purified by distillation.

One convenient and presently preferred procedure for the preparation of the quaternary ammonium compound is to separately prepare the ester and the quaternizing agent as solutes in the same highly polar solvent, acetonitrile being one presently particularly preferred example. The mole ratio of quaternary ammonium compound to the quaternizing agent is preferably about 1:1. Such a solution is then heated at reflux for a time in the range of about 1 to about 2 hours. The reaction mixture is then concentrated by solvent evaporation to yield a viscous oil or a crystalline solid. The product can be used without further purification for the next step in the syntheses, or the product can be purified by recrystallization, for example, from a ketone, such as 2-butanone, or the like, followed by washing and drying.

One convenient and presently preferred procedure for preparation of the quaternary ammonium organic salt from the intermediate halide is to dissolve the ion exchange agent in an aqueous solution. To this solution is added a second aqueous solution containing the quaternary ammonium salt intermediate. The mole ratio of such salt to such ion exchange agent should be about 1:1. Typically, a precipitate is formed immediately which is in the form of an oil. This precipitate is collected, water washed (preferably with distilled or deionized water), and then dissolved in a water immiscible organic solvent, such as methylene dichloride, or the like. The water layer is separated, the organic layer is dried over MgSO<sub>4</sub>, or the like, and the product thereby concentrated. The resulting product can be recrystallized from an alkanol, such as isopropanol, or the like, or a ketone, such as 2-butanone, or the like, if desired.

### (D) Toners And Toner Preparation

The quaternary ammonium salts of the present invention are incorporated into toner particles. For present purposes, toner particles can be regarded as being preferably comprised on a 100 weight percent basis of:

(a) about 0.5 to about 10 weight percent of at least one quaternary ammonium salt;

(b) about 75 to about 97.5 weight percent of a thermoplastic polymer; and

(c) about 2 to about 15 weight percent of a colorant.

The size of the toner particles is believed to be relatively unimportant from the standpoint of the present invention; rather the exact size and size distribution is influenced by the end use application intended. So far as now known, the toner particles of this invention can be used in all known electrophotographic copying processes. Typically and illustratively, toner particle sizes

range from about 0.5 to about 100 microns, preferably from about 4 to about 35 microns.

The properties of a thermoplastic polymer employed as a toner matrix phase can vary widely. Typically and preferably, toner polymers have a glass transition temperature in the range of about 50° to about 120° C. and a melting temperature in the range of about 65° to about 200° C. Preferably, such a polymer has a number average molecular weight in the range of about 1,000 to about 10,000. The weight average molecular weight can vary, but preferably is in the range of about 10<sup>4</sup> to about 10<sup>6</sup>. Typical examples of such polymers include polystyrene, polyacrylates, polyesters, polyamides, polyolefins, polycarbonates, phenol formaldehyde condensates, alkyl resins, polyvinylidene chlorides, epoxy resins, various copolymers of the monomers used to make these polymers, such as polyesteramides, acrylonitrile copolymers with monomers, such as styrene, acrylics, and the like.

Preferably, thermoplastic polymers used in the practice of this invention are substantially amorphous. However, mixtures of polymers can be employed, if desired, such as compatible mixtures of substantially amorphous polymers with substantially crystalline polymers.

Presently preferred polymers for use in toner powders are polyesters. The structure of the polyester polymer can vary widely, and mixtures of different polyesters can be employed. Polyesters and methods for making such are generally known to the prior art. One presently more preferred polyester is polyethylene terephthalate, such as polyethylene terephthalate having an inherent viscosity in the range of about 0.25 to about 0.35 in methylene chloride solution at a concentration of about 0.25 grams of polymer per 100 milliliters of solution. In general, preferred polyesters have a glass transition temperature ( $T_g$ ) in the range of about 50° to about 120° C. and a melting temperature ( $T_m$ ) in the range of about 65° to about 200° C.

An optional but preferred starting material for inclusion in such a blend is a colorant (pigment or dye). Suitable dyes and pigments are disclosed, for example, in U.S. Pat. No. 31,072, and in U.S. Pat. Nos. 4,140,644; 4,416,965; 4,414,152; and 2,229,513. One particularly useful colorant for the toners to be used in black and white electrophotographic copying machines is carbon black. When employed, colorants are generally employed in quantities in the range of about 1 to about 30 weight percent on a total toner powder weight basis, and preferably in the range of about 1 to about 8 weight percent.

The quaternary ammonium salts of the present invention are compatible with conventional charge control agents and other toner additives. If desired, a conventional charge control agent can be additionally incorporated into a toner particle composition. Examples of such charge control agents for toner usage are described in, for example, U.S. Pat. Nos. 3,893,935; 4,079,014; 4,323,634; and British Patent Nos. 1,501,065 and 1,420,839. If used, charge control agents are preferably employed in small quantities, such as an amount in the range of about 0.1 to about 5 weight percent on a total toner composition weight basis, and preferably in the range of about 0.1 to about 3 weight percent.

Toner compositions, if desired, can also contain other additives of the types which have been heretofore employed in toner powders, including leveling agents, surfactants, stabilizers, and the like. The total quantity of such additives can vary. A present preference is to

employ not more than about 10 weight percent of such additives on a total toner powder composition weight basis.

Various procedures are known to the art for incorporating additives, such as the quaternary ammonium salts of the present invention, colorants, or the like, into a desired polymer. For example, a preformed mechanical blend of particulate polymer particles, quaternary ammonium salts, colorants, etc., can be roll milled or extruded at a temperature above the melt blending temperature of the polymer to achieve a uniformly blended composition. Thereafter, the cooled composition can be ground and classified, if desired, to achieve a desired toner powder size and size distribution.

Preferably, prior to melt blending, the toner components, which preferably are preliminarily placed in a particulate form, are blended together mechanically. With a polymer having a  $T_g$  or a  $T_m$  within the ranges above indicated, a melt blending temperature in the range of about 90° to about 160° C. is suitable using a roll mill or extruder. Melt blending times (that is, the exposure period for melt blending at elevated temperatures) are in the range of about 1 to about 60 minutes. After melt blending and cooling, the composition can be stored before being ground. Grinding can be carried out by any convenient procedure. For example, the solid composition can be crushed and then ground using, for example, a fluid energy or jet mill, such as described in U.S. Pat. No. 4,089,472. Classification, if employed, can be conventionally accomplished using one or two steps.

In place of melt blending, the polymer can be dissolved in a solvent and the additives dissolved and/or dispersed therein. Thereafter, the resulting solution or dispersion can be spray dried to produce particulate toner powders.

Limited coalescence polymer suspension procedures, are particularly useful for producing small sized, uniform toner particles, such as toner particles under about 10 microns in size.

Toner powders of this invention preferably have a fusing latitude temperature in the range of about 275° to about 400° F., although toner powders with higher and lower fusing temperatures can be prepared and used. Toner powders of this invention characteristically display excellent paper adhesion characteristics. Typically, toner powders of this invention have a paper adhesion index value in the range of about 30 to about 100, although toner powders with lower such values can be prepared and used. Paper adhesion index values of toner powders of this invention are characteristically higher than those of toner powders prepared with the same polymer and additives but not containing a quaternary ammonium salt of this invention.

When the polymer employed in a toner powder of this invention is a polyester, the ester group containing quaternary ammonium salts used in this invention display superior ester compatibility therewith.

The invention is further illustrated by the following Examples. In these Examples, all melting points and boiling points are uncorrected. NMR (nuclear magnetic resonance) spectra were obtained with a Varian Gemini-200 NMR spectrometer. All elemental analyses were performed by mass spectroscopy. Unless otherwise indicated, all starting chemicals were commercially obtained.

## EXAMPLE 1

## 2-(N,N-Dimethylamino)ethyl 4-methylvalerate

A solution of 67.31 g (0.50 mol) of 4-methylvaleryl chloride in 300 ml of methylene chloride was added to a solution of 44.57 g (0.50 mol) of 2-dimethylaminoethanol, 20.0 g (0.50 mol) of sodium hydroxide and 300 ml of water in a stream via a dropping funnel while maintaining rapid stirring. The reaction was exothermic and was stirred for an additional 20 minutes. The organic layer was then separated, washed with water, dried over  $MgSO_4$  and concentrated to an oil. Distillation of the oil gave 56.8 g of product;  $bp = 70^\circ C./0.80$  mm.

Anal. Calcd. for  $C_{10}H_{21}NO_2$ : C, 64.13; H, 11.30; N, 7.48; Found: C, 59.78; H, 10.94; N, 6.51.

## EXAMPLE 2

## 2-(N,N-Dimethylamino)ethyl benzoate

A solution of 70.29 g (0.50 mol) of benzoyl chloride in 500 ml of methylene chloride was added to a solution of 44.57 g (0.50 mol) of 2-dimethylaminoethanol, 20.0 g (0.50 mol) of sodium hydroxide and 500 ml of water over 15 minutes with rapid stirring. Stirring was continued for 3.25 hours after which the organic layer was separated, washed with water, dried over  $MgSO_4$  and concentrated. Distillation of the residue gave 59.5 g of product;  $bp = 102^\circ-8^\circ C./0.50$  mm.

Anal. Calcd. for  $C_{11}H_{15}NO_2$ : C, 68.37; H, 7.82; N, 7.25; Found: C, 66.11; H, 7.89; N, 7.25.

## EXAMPLE 3

## 2-(N,N-Dimethylamino)ethyl 2-ethyl hexanoate

The title compound was prepared by the procedure of Example 1.

## EXAMPLE 4

## 2-(N,N-Dimethylamino)ethyl cyclohexanoate

The title compound was prepared by the procedure of Example 1.

## EXAMPLE 5

## 2-(N,N-Dimethylamino)ethyl myristate

A solution of 91.35 g (0.40 mol) of myristic acid, 35.7 g (0.40 mol) of 2-dimethylaminoethanol, 0.5 g of p-toluenesulfonic acid and a suitable volume of toluene was heated at reflux for approximately 48 hours in a 1-neck 3 liter flask equipped with Dean-Stark trap and condenser. At the end of this time, 7.0 ml of water had collected in the trap. The solution was cooled, stirred with  $K_2CO_3$ , filtered and concentrated. The residue was distilled to give 75.0 g of product;  $bp = 145^\circ-50^\circ C./0.050$  mm.

## EXAMPLE 6

## 2-(N,N-Dimethylamino)ethyl 4-chlorobenzoate

The title compound was prepared by the procedure of Example 1.

## EXAMPLE 7

## 2-(N,N-Dimethylamino)ethyl 4-methoxybenzoate

The title compound was prepared by the procedure of Example 1.

The acid or acid chloride starting materials and the analytical data for the ester products are shown in Table I below for Examples 1-7.

TABLE I

## 2-(N,N-DIMETHYLAMINO) ETHYL ESTERS



| Ex. No. | Starting acid Or Acid Chloride | Identity of $R_1$         | bp, C/mm                            | Analyses |       |       |       |                                      |
|---------|--------------------------------|---------------------------|-------------------------------------|----------|-------|-------|-------|--------------------------------------|
|         |                                |                           |                                     | Calcd    |       | Found |       |                                      |
| C       | H                              | N                         | Cl                                  | C        | H     | N     | Cl    |                                      |
| 1       | 4-methyl-valeroyl chloride     | $(CH_3)_2CHCH_2CH_2-$     | 70/0.8                              | 64.13    | 11.30 | 7.48  |       | 59.78 10.94 6.51                     |
| 2       | benzoyl chloride               |                           | 102-8/0.5                           | 68.37    | 7.82  | 7.25  |       | 66.11 7.89 7.25                      |
| 3       | 2-ethyl hexanoyl chloride      | $CH_3(CH_2)_3CH(C_2H_5)-$ | 75-8/0.75                           | 66.9     | 11.7  | 6.5   |       | 65.4 10.8 6.3                        |
| 4       | cyclohexane-carbonyl chloride  |                           | 78/0.65<br>88-9/0.50 <sup>(1)</sup> | 66.29    | 10.62 | 7.03  |       | 64.51 10.07 7.20<br>66.38 10.99 7.49 |
| 5       | myristic acid                  | $CH_3(CH_2)_{12}-$        | 145-50/0.5                          | 72.19    | 12.45 | 4.68  |       | 72.34 12.06 3.98                     |
| 6       | 4-chlorobenzoyl chloride       |                           | 122-8/0.50                          | 58.03    | 6.20  | 6.15  | 15.57 | 57.50 6.29 6.0 14.84                 |

TABLE I-continued

## 2-(N,N-DIMETHYLAMINO) ETHYL ESTERS



| Ex.<br>No. | Starting acid Or<br>Acid Chloride | Identity of R <sub>1</sub> | bp. C/mm    | Analyses              |                       |   |   |   |
|------------|-----------------------------------|----------------------------|-------------|-----------------------|-----------------------|---|---|---|
|            |                                   |                            |             | Calcd                 | Found                 | C | H | N |
| 7          | 4-methoxy benzoyl<br>chloride     |                            | 128-40/0.30 | 64.55<br>7.67<br>6.27 | 64.59<br>7.46<br>6.13 |   |   |   |

(1) Intermediate ester distilled twice before analysis

## EXAMPLE 8

## N-(4-Methylvaleroxyethyl)-N,N-dimethylbenzylammonium chloride

A solution of 46.83 g (0.25 mol) of 2-(N,N-dimethylamino)ethyl-4-methylvalerate (prepared as described in Example 1) and 31.65 g (0.25 mol) of benzyl chloride in 250 ml of acetonitrile was heated at reflux for 1.25 hours. The reaction mixture was then concentrated to a viscous oil and used in the ion exchange step with no further purification.

## EXAMPLE 9

## N-(Benzoyloxyethyl)-N,N-dimethylbenzylammonium chloride

A solution of 57.96 g (0.30 mol) of 2-(N,N-dimethylamino)ethyl benzoate (prepared as described in Example 2), 37.98 g (0.30 mol) of benzyl chloride and 500 ml of acetonitrile was heated at reflux for 2 hours. The reaction mixture was concentrated to a white solid which was then washed with ether and recrystallized from acetonitrile. The yield of product was 69.0 g; mp = 164°-6° C.

## EXAMPLE 10

## N-(2-Ethylhexanoyloxyethyl)-N,N-dimethylbenzylammonium chloride

The title compound was prepared by the procedure of Example 8.

## EXAMPLE 11

## N-(Cyclohexanoyloxyethyl)-N,N-dimethylbenzylammonium chloride

The title compound was prepared by the procedure of Example 8.

## EXAMPLE 12

## N-(Myristyloxyethyl)-N,N-dimethylbenzylammonium chloride

The title compound was prepared by the procedure of Example 8.

## EXAMPLE 13

## N-(4-Chlorobenzoyloxyethyl)-N,N-dimethylbenzylammonium chloride

The title compound was prepared by the procedure of Example 9.

## EXAMPLE 14

## N-(4-Methoxybenzoyloxyethyl)-N,N-dimethylbenzylammonium chloride

The title compound was prepared by the procedure of Example 9.

The ester starting materials and the analytical data for the quaternary ammonium chloride products are shown in Table II below for Examples 8-14.

TABLE II

## N-(2-ACYLOXYETHYL)-N,N-DIMETHYL BENZYLAMMONIUM CHLORIDES\*



| Ex.<br>No. | Identity of R <sub>1</sub>                                          | mp. C | Analyses |       |   |   |   |
|------------|---------------------------------------------------------------------|-------|----------|-------|---|---|---|
|            |                                                                     |       | Calcd    | Found | C | H | N |
| 8          | (CH <sub>3</sub> ) <sub>2</sub> CHCH <sub>2</sub> CH <sub>2</sub> - | oil   |          |       |   |   |   |

9 164-6



TABLE II-continued

## N-(2-ACYLOXYETHYL)-N,N-DIMETHYLBENZYLAMMONIUM CHLORIDES\*



| Ex.<br>No. | Identity of R <sub>1</sub>                                                          | mp, C     | Analyses              |                       |   |   |   |
|------------|-------------------------------------------------------------------------------------|-----------|-----------------------|-----------------------|---|---|---|
|            |                                                                                     |           | Calcd                 | Found                 | C | H | N |
| 10         | CH <sub>3</sub> (CH <sub>2</sub> ) <sub>3</sub> CH(C <sub>2</sub> H <sub>5</sub> )— | oil       |                       |                       |   |   |   |
| 11         |                                                                                     | oil       |                       |                       |   |   |   |
| 12         | CH <sub>3</sub> (CH <sub>2</sub> ) <sub>12</sub> —                                  | oil       |                       |                       |   |   |   |
| 13         |                                                                                     | 196 dec   | 61.03 5.97 3.95 20.01 | 60.63 5.86 4.02 20.05 |   |   |   |
| 14         |                                                                                     | 195-6 dec | 65.23 6.91 4.00 10.13 | 64.97 6.77 4.13 11.43 |   |   |   |

\*Quaternizing agent was benzyl chloride

## EXAMPLE 15

## N-(4-Methylvaleryloxyethyl)-N,N-dimethylbenzylammonium m-nitrobenzenesulfonate

A hot solution (300 ml) of 56.29 g (0.25 mol) of sodium m-nitrobenzenesulfonate in water was added to a solution (300 ml) of 78.48 g (0.25 mol) of N-(4-methylvaleryloxyethyl)-N,N-dimethylbenzylammonium chloride prepared as described in Example 8) in water. An oily precipitate formed immediately which crystallized on cooling. The solid was collected, washed with water and dissolved in methylene chloride. The water layer was separated and the organic layer was dried over MgSO<sub>4</sub> and concentrated. Recrystallization of the solid residue from isopropanol gave 81.6 g of product; mp=106°-8° C. Anal. Calcd. for C<sub>23</sub>H<sub>32</sub>N<sub>2</sub>O<sub>7</sub>; C, 57.84; H, 6.71; N, 5.83; S, 6.67; Found: C, 57.26; H, 6.53; N, 5.90; S, 6.85.

## EXAMPLE 16

## N-(Benzoyloxyethyl)-N,N-dimethylbenzylammonium m-nitrobenzenesulfonate

A solution of 45.03 g (0.20 mol) of sodium m-nitrobenzenesulfonate in 200 ml of water was added to a solution of 63.97 g (0.20 mol) of N-(benzoyloxyethyl)-N,N-dimethylbenzylammonium chloride (prepared as described in Example 9) in 250 ml of water. An oily precipitate immediately formed. The water was decanted from the oil and fresh water was added. After standing overnight, the oil was taken up in methylene chloride. The water layer was separated and the organic layer was dried over MgSO<sub>4</sub> and concentrated to an oil which crystallized. The solid was recrystallized

from 2-butanone, collected, washed with ether and dried. The yield of product was 36.0 g; mp=104°-6° C.

Anal. Calcd. for C<sub>24</sub>H<sub>26</sub>N<sub>2</sub>O<sub>7</sub>S  
C, 59.25; H, 5.39; N, 5.76; S, 6.59;  
Found: C, 58.90; H, 5.34; N, 5.62; S, 6.76.

## EXAMPLE 17

## 45 N-(2-Ethylhexanoxyloxyethyl)-N,N-dimethylbenzylammonium m-nitrobenzenesulfonate

The title compound was prepared by the procedure of Example 16.

## EXAMPLE 18

## N-(cyclohexanoyloxyethyl)-N,N-dimethylbenzylammonium m-nitrobenzenesulfonate

The title compound was prepared by the procedure of Example 16.

## EXAMPLE 19

## N-(myristyloxyethyl)-N,N-dimethylbenzylammonium m-nitrobenzenesulfonate

60 The title compound was prepared by the procedure of Example 16.

## EXAMPLE 20

## N-(4-chlorobenzoyloxyethyl)-N,N-dimethylbenzylammonium m-nitrobenzenesulfonate

The title compound was prepared by the procedure of Example 16.

## EXAMPLE 21

**N-(4-methoxybenzoyloxyethyl)-N,N-dimethylbenzylammonium m-nitrobenzenesulfonate**

The title compound was prepared by the procedure of Example 16.

The quaternary ammonium chloride starting materials and the analytical data for the quaternary ammonium m-nitrobenzenesulfonate salt products are shown in Table III below for Examples 15-21.

## EXAMPLE 23

**N,N-Bis(2-cyclohexanoyloxyethyl)-N-methylbenzylammonium chloride**

A solution of 28.5 g (0.084 mol) of N,N-bis(2-cyclohexanoyloxyethyl)methylamine (prepared as described in Example 22), 10.63 g (0.084 mol) of benzyl chloride and 200 ml of acetonitrile was heated at reflux for 2.5 hours and concentrated to an oil. Ether was added to the oil which induced crystallization. The

TABLE III

**N-(2-ACYLOXYETHYL)-N,N-DIMETHYLBENZYLAMMONIUM M-NITROBENZENESULFONATES\***



## Analyses

| Ex.<br>No. | Identity of R <sub>1</sub>                                                          | mp. C       | Calcd |      |      |      |      | Found |      |      |      |      |
|------------|-------------------------------------------------------------------------------------|-------------|-------|------|------|------|------|-------|------|------|------|------|
|            |                                                                                     |             | C     | H    | N    | Cl   | S    | C     | H    | N    | Cl   | S    |
| 15         | (CH <sub>3</sub> ) <sub>2</sub> CHCH <sub>2</sub> CH <sub>2</sub> -                 | 106-8       | 57.48 | 6.71 | 5.83 |      | 6.67 | 57.26 | 6.53 | 5.90 |      | 6.85 |
| 16         |                                                                                     | 104-6       | 59.25 | 5.39 | 5.76 |      | 6.59 | 58.90 | 5.34 | 5.62 |      | 6.76 |
| 17         | CH <sub>3</sub> (CH <sub>2</sub> ) <sub>3</sub> CH(C <sub>2</sub> H <sub>5</sub> )- | —           | 59.04 | 7.13 | 5.51 |      | 6.30 | 59.32 | 7.02 | 5.48 |      | 6.31 |
| 18         |                                                                                     | 97-9        | 58.5  | 6.54 | 6.51 |      | 6.51 | 58.5  | 6.39 | 6.58 |      | 6.58 |
| 19         | CH <sub>3</sub> (CH <sub>2</sub> ) <sub>12</sub> -                                  | 54-7        | 62.81 | 8.16 | 4.73 |      | 5.41 | 63.27 | 8.36 | 4.09 |      | 4.54 |
| 20         |                                                                                     | 123.5-125.5 | 55.33 | 4.84 | 5.38 | 6.80 | 6.15 | 55.45 | 4.87 | 5.20 | 7.39 | 6.30 |
| 21         |                                                                                     | 152-153     | 58.13 | 5.46 | 5.42 |      | 6.21 | 58.18 | 5.56 | 5.42 |      | 6.71 |

\*Iow exchange agent was sodium m-nitrobenzenesulfonate

## EXAMPLE 22

**N,N-Bis(2-cyclohexanoyloxyethyl)methylamine**

A solution of 73.31 g (0.05 mol) cyclohexanecarbonyl chloride in 200 ml of methylene chloride was added to a solution of 29.79 g (0.25 mol) of N-methyldiethanolamine, 20.0 g (0.50 mol) of sodium hydroxide and 200 ml of water over approximately 1 minute. The reaction was exothermic requiring the use of a reflux condenser. The reaction mixture was stirred for another 45 minutes after which the organic layer was separated, washed with water, dried over MgSO<sub>4</sub> and concentrated. The residue was distilled to give product, bp=192°-9° C./0.30 mm.

Anal. Calcd for C<sub>19</sub>H<sub>33</sub>NO<sub>4</sub>: C,67.22;H, 9.80;N,4.13; Found: C,67.45;H,10.05;N,4.31.

white solid was collected, washed two times with ether and recrystallized from 2-butanone. The yield of product was 8.3 g; mp=143.5°-4.5° C.

Anal. Calcd for C<sub>26</sub>H<sub>40</sub>ClNO<sub>4</sub>: C,67.01;H,8.65;Cl,7.61;N,3.01; Found: C,66.86;H,8.51;Cl,7.51;N,2.93.

## EXAMPLE 24

**N,N-Bis(2-cyclohexanoyloxyethyl)-N-methyl-benzylammonium m-nitrobenzenesulfonate**

A solution of 3.38 g (0.015 mol) of sodium m-nitrobenzenesulfonate in 15 ml of water was added to a solution of 7.0 g (0.015 mol) of N,N-bis(2-cyclohexanoyloxyethyl)-N-methylbenzylammonium chloride (prepared as described in Example 23) in 50 ml of water. An oily precipitate immediately formed. The oil was

rinsed twice with water, dissolved in methylene chloride, dried over  $MgSO_4$  and concentrated. The resultant oil was crystallized with P-513 ligoine and warmed. The crystals were collected, washed with ether, dried and recrystallized from 2-butanone. The yield of product was 2.64 g; mp = 123°-4.5° C.

Anal. Calcd for  $C_{23}H_{44}N_2O_9S$ : C, 60.74; H, 7.01; N, 4.43; S, 5.50; C, 60.37; H, 6.93; N, 4.34; S, 5.17.

### EXAMPLE 25

#### Bis(2-dimethylaminoethyl) terephthalate

A solution of 40.60 g (0.20 mol) of terephthaloyl chloride in 200 ml methylene chloride was gradually added to a solution of 35.66 g (0.40 mol) of 2-dimethylaminoethanol, 16.0 g (0.40 mol) of sodium hydroxide and 200 ml of water and stirred rapidly. The reaction was exothermic and achieved reflux. The mixture was stirred for another 1.75 hours after which the organic layer was separated, washed with water, dried over  $MgSO_4$  and concentrated to an oil.

Anal. Calcd for  $C_{16}H_{24}N_2O_4$ : C, 62.32; H, 7.84; N, 9.08; Found: C, 60.74; H, 8.56; N, 9.5.

### EXAMPLE 26

#### Bis(2-(N,N-dimethylbenzylammonium)ethyl) terephthalate dichloride

A solution of 30.84 g (0.10 mol) of bis(2-dimethylaminoethyl) terephthalate and 25.32 g (0.20 mol) of benzyl chloride was heated on a steam bath. Within a few minutes, the mixture solidified. The resultant caked solid was washed with acetonitrile and used in the next step without further purification.

### EXAMPLE 27

#### Bis(2-(N,N-dimethyl benzylammoniummethyl) terephthalate bis-(m-nitrobenzenesulfonate)

A solution of 56.16 g (0.01 mol) of the crude bis(2-N,N-dimethylbenzylammonium)ethyl)terephthalate prepared as described in Example 26 in 200 ml of water was added to a solution of 45.02 g (0.20 mol) of sodium m-nitrobenzenesulfonate in 200 ml of water. An oily precipitate immediately formed. The aqueous phase was decanted and the residue was washed several times with water. Ethyl acetate was added to the oil and after standing the oil crystallized. The solid was collected, washed with ether and recrystallized twice from acetonitrile to give 32.7 g (36.5%) of a product whose melting point was 170°-1° C.

Anal. Calcd for  $C_{42}H_{46}N_4O_{14}S_2$ : Found: C, 56.37; H, 5.18; N, 6.26; S, 7.17; C, 56.13; H, 5.05; N, 6.21; S, 7.57.

### EXAMPLE 28

#### Poly(2-dimethylaminoethyl methacrylate)

A solution of 50.0 g (0.318 mol) of N,N-dimethylaminoethyl methacrylate in 450 g of DMF was purged with nitrogen. Azobisisobutyronitrile (0.50 g) was added and the solution was heated in a 60° C. bath for 53.6 hours. The resultant polymer was used in the next step without isolation.

### EXAMPLE 29

#### Poly(2-(N,N-dimethyl aminobenzylammonium)ethyl methacrylate chloride)

The solution of poly(2-dimethylaminoethyl methacrylate) prepared in the preceding Example 28 in dimethylformamide was treated with 40.26 g (0.318 mol) of benzyl chloride and heated under nitrogen in a 60° C. bath for 4 hours. A viscous oil precipitated and was allowed to stand for 10 days. Acetone was added to the mixture to harden the polymer which was then collected and used in the next step with no further purification.

### EXAMPLE 30

#### Poly(2-(N,N-dimethylbenzyl ammonium)ethyl methacrylate m-nitrobenzenesulfonate)

The poly(2-(N,N-dimethylaminobenzylammonium)ethyl methacrylate chloride prepared in the preceding Example 29 was dissolved in 1 liter of water and to it was added a solution of 71.6 g (0.318 mol) of sodium m-nitrobenzenesulfonate in 500 ml of water. A polymer immediately precipitated. The aqueous phase was decanted and the polymer was allowed to stand overnight in water. The water was decanted and the polymer was washed with acetone and then ether, and finally dried. The polymer was dissolved in DMF and reprecipitated into ether. The gummy precipitate was isolated, washed again with ether and dried. The structure was confirmed by NMR although the polymer was strongly contaminated with DMF.

### EXAMPLES 30-33

The procedure for Example 16 is repeated except that, in place of sodium m-nitrobenzenesulfonate, one equivalent of each of the ion exchange salts shown in the following Table IV in such an aqueous solution is added to the starting quaternary ammonium chloride solution. The structure of the cation formed in, and the melting point of, each salt so recovered and recrystallized is shown in Table IV. For comparison purposes, the melting point of the product of Example 16, and the melting point of the starting compound of Example 8 are included in Table IV.

TABLE IV

#### N-(2-BENZOYLOXYETHYL)-N,N-DIMETHYLBENZYLAMMONIUM SALTS



| Ex. No. | Starting Ion Exchange Agent    | Identity of Y- in Formula    | Melting Point °C. |
|---------|--------------------------------|------------------------------|-------------------|
| 8       |                                | $Cl^-$                       | 170-172           |
| 16      | sodium m-nitrobenzenesulfonate | $SO_3^-$ (with $NO_2$ group) | 104-6             |
| 31      | sodium tetraphenylborate       | $B(OPh_3)_4^-$               | 194-6             |
| 32      | sodium dicyanamide             | $N(CN)_2^-$                  | (amorphous)       |

TABLE IV-continued

| N-(2-BENZOYLOXYETHYL)-N,N-DIMETHYLBENZYLAMMONIUM SALTS                            |                                             |                                                                                                                   |
|-----------------------------------------------------------------------------------|---------------------------------------------|-------------------------------------------------------------------------------------------------------------------|
|  |                                             |                                                                                                                   |
| Starting Ion<br>Ex. No.<br>33                                                     | Exchange Agent<br>sodium p-toluenesulfonate | Identity of Y-<br>in Formula<br> |
|                                                                                   |                                             | Melting Point °C.<br>110-112                                                                                      |

## EXAMPLES 34-36

## Toner Powder Preparation

An amorphous branched polyester comprised of a condensate of dimethylterephthalate (87 mole %), dimethylglutarate (13 mole %), 1,2-propanediol (95 mole %) and glycerol (5 mole %) having a  $T_g$  of 63°C. and a number average molecular weight of about 3000 was prepared using a conventional polycondensation technique. This polymer was preliminarily ground into particles having a size in the range of about 1/16", and such particles are blended with various additives as 30 individually identified in the following Table V to produce various blends as shown in such Table.

TABLE V

| Toner Composition (Dry Weight Basis) |                           |           |                   |                  |                   |                  |
|--------------------------------------|---------------------------|-----------|-------------------|------------------|-------------------|------------------|
| Component                            | ID No.                    | Component | Blend Ex. 34      |                  | Blend Ex. 35      |                  |
|                                      |                           |           | wt % <sup>5</sup> | pph <sup>6</sup> | wt % <sup>5</sup> | pph <sup>6</sup> |
| 1                                    | Polyester                 |           | 90.66             | 100.0            | 91.74             | 100.0            |
| 2                                    | Carbon Black <sup>3</sup> |           | 4.53              | 5.0              | 4.59              | 5.0              |
| 3                                    | LSA <sup>4</sup>          |           | 3.63              | 4.0              | 3.67              | 4.0              |
| 4                                    | Charge Control Agent      |           | 1.18 <sup>1</sup> | 1.3              | (none)            | (none)           |
| TOTAL                                |                           |           | 100               | 110.3            | 100               | 109.0            |
|                                      |                           |           | 100               | 100              | 100               | 110.3            |

Table V Footnotes:

<sup>1</sup>Charge Control Agent<sup>2</sup>The charge control agent was the compound identified in Example 16 above.<sup>3</sup>The carbon black was "Regal TM 300" obtained commercially from Cabot Corporation.<sup>4</sup>The LSA was a polyester/polydimethylsiloxane block copolymer as described in U.S. Pat. No. 4,758,491.<sup>5</sup>Weight percent on a total blend composition basis.<sup>6</sup>Parts by weight.

The carbon black was "Regal TM 300" as in Examples 34-36. The charge control agent was methyltriphenyl phosphonium tosylate.

This blend was extruded on a twin screw extruder cooled, crushed, ground and classified to produce a toner powder.

#### EXAMPLES 43-44

##### Toner Powder Preparation

The polyester described in Examples 34-36 was additionally compounded with various additives as individually identified in the following Table VIII.

TABLE VIII

| Component ID. No. | Component                   | Toner Composition (Dry Weight Basis) |                           |
|-------------------|-----------------------------|--------------------------------------|---------------------------|
|                   |                             | Blend Comp. Ex. 43<br>pph            | Blend Comp. Ex. 44<br>pph |
| 1                 | polyester                   | 100                                  | 100                       |
| 2                 | yellow pigment              | 3                                    | 3                         |
| 3                 | <u>Charge control agent</u> |                                      |                           |
|                   | A                           | 1.5                                  |                           |
|                   | B                           |                                      | 1.5                       |

Charge control agent A was that used in Example 34; this charge control agent and the formulation of Example 44 were utilized for comparative purposes. Charge control agent B was the compound identified in Example 16 above.

Each blend was roll milled on the same roll mill as used in Examples 35-37, cooled, crushed, ground and classified to produce a toner powder product.

#### EXAMPLES 45-48

##### Toner Powder Preparation

A styrene butylacrylate copolymer was obtained by limited coalescence polymerization and blended with various additives as identified in the following TABLE IX.

TABLE IX

| Component ID No. | Component                       | Toner Composition (Dry Weight Basis) |     |
|------------------|---------------------------------|--------------------------------------|-----|
|                  |                                 | Concentration                        | pph |
| 1                | Styrene butylacrylate copolymer | 100                                  |     |
| 2                | Carbon black                    | 3                                    |     |
| 3                | Charge Control Agent            |                                      |     |
|                  | Formulation of Ex. 45           | 1                                    |     |
|                  | Formulation of Ex. 46           | 1                                    |     |
|                  | Formulation of Ex. 47           | 2                                    |     |
|                  | Formulation of Ex. 48           | 1                                    |     |

The carbon black was "Regal TM 300" as in Examples 34-36. The charge control agent used for the formulation of Example 45 was as in Example 34. The formulation of Example 45 was utilized for comparative purposes. The charge control agent used for the formulation of Examples 46 and 47 was the compound identified in Example 18 above. The charge control agent used for the formulation of Example 48 was the compound identified in Example 16 above.

Each of such formulations was roll milled, cooled, crushed, ground and classified to produce a toner powder product.

#### EXAMPLE 49

##### Toner $T_g$

To determine if the quaternary ammonium salt compounds were plasticizing the toner and thereby affecting fusing, the  $T_g$  of each of the toner powders of Examples 37-41 above was measured. The results were shown in the following Table X.

TABLE X

| Toner Glass Transition Temperature |  |                |
|------------------------------------|--|----------------|
| Toner ID<br>Ex. No.                |  | $T_g$<br>(°C.) |
| 37                                 |  | 60.6           |
| 38                                 |  | 62.2           |
| 39                                 |  | 61.8           |
| 40                                 |  | 60.9           |
| 41                                 |  | 60.8           |

Since this data shows that the toner powders containing the compounds of Examples 16 and 18 had  $T_g$  values which were equivalent to or slightly above, the  $T_g$  value for a toner powder containing the charge agent of Example 34, it was concluded that the quaternary ammonium salt compounds are not acting as plasticizers in toner particles.

#### EXAMPLE 50

##### Fusing And Adhesion

Each of the polyester-based toner powders of Examples 34-36 was evaluated on a fusing breadboard consisting of a fusing roller coated with a fluorocarbon elastomer (available commercially under the designation Viton TM from E. I. du Pont de Nemours & Co.) engaged at constant speed and pressure onto a backup roller coated with a polytetrafluoroethylene (available commercially as Silverstone TM from E. I. duPont de Nemours & Co. Both rollers had their circumferential surfaces coated by hand using a release oil (available commercially under the designation "DC200 oil" from Dow Corning Company).

Six longitudinally extending stripes of toner were applied to various receiver sheets which were then run through the fusing breadboard.

The receiver sheets were:

- Husky TM paper, an acidic paper, available commercially from Weyerhaeuser Company;
- Kodak TM DP paper, available commercially from Eastman Kodak Company; and
- Hammermill TM 9000 DP, an alkaline paper available commercially from the Hammermill Company.

The adhesion index (A.I.) and crack width at various temperatures for each toner powder were determined and used as an indication of fusing performance. The results are shown for the Hammermill.

TABLE XI

| Temperature<br>°F. | Adhesion Index at Various Temperatures |        |        |
|--------------------|----------------------------------------|--------|--------|
|                    | Adhesion Index (A.I.) of Toner         |        |        |
|                    | Ex. 35                                 | Ex. 37 | Ex. 41 |
| 275                | 10                                     | 5      | 10     |
| 300                | 5                                      | 10     | 20     |
| 325                | 30                                     | 12     | 35     |
| 350                | 62                                     | 30     | 80     |
| 375                | 100                                    | 25     | 100    |

The toner of Example 35 contained no charge agent, the toner of Example 37 contained the charge agent of

